

## UNITED STATES PATENT OFFICE.

HUGH RODMAN, OF OAKMONT, AND EARL E. BOREN, OF SWISSVALE, PENNSYLVANIA,  
ASSIGNORS TO RODMAN CHEMICAL COMPANY, A CORPORATION OF PENNSYLVANIA.

## DECOLORIZING MATERIAL AND PROCESS OF MAKING SAME.

No Drawing.

Application filed June 4, 1918. Serial No. 238,162.

*To all whom it may concern:*

Be it known that we, HUGH RODMAN, a citizen of the United States, and a resident of Oakmont, Pennsylvania, and EARL E. BOREN, a citizen of the United States, and a resident of Swissvale, Pennsylvania, have made a new and useful Invention in Decolorizing Material and Process of Making Same, of which the following is a specification.

This invention relates to a special material having unusual properties as a filtering and decolorizing medium and to the method of producing this material.

In Patent 1,420,754, granted June 27, 1922, to Hugh Rodman, one of the joint inventors herein named, a new product is described and claimed, which is produced by heating rotted coal. Rotted coal, as the term is herein employed, refers to the coal in that portion of coal veins which, ordinarily hard and normal, has rotted or deteriorated so that the characteristics of the coal have completely altered. This rotted coal exists near the surface of the ground under which the coal lies, and seems to be due to the slow disintegration of the firm coal, and apparently results in some way from the thin cover over the coal. This rotted coal is a laminated, friable material holding about thirty per cent of water, which produces no smoke or coke when heated (though the coal in the same seam farther back under the hill will both smoke and coke) and which is largely soluble in weak alkalies.

We have discovered that when this rotted coal is highly heated, and treated as herein-after described, a char is obtained having valuable characteristics in the way of decolorizing oils and other liquids. We have produced a fair decolorizing material by simply passing the raw rotted coal through a rotary kiln heated to about 1800 degrees Fahrenheit, some care being taken to see that the material was in contact with hot air for at least a short period after most of the volatile matter had been distilled off. We have produced better decolorizing material by first charring the rotted coal and then keeping it in contact with highly superheated steam for a period of time, the duration of which depends upon the relative volume of the steam and the char and also upon the fineness of the individual char par-

ticle. We have also experimented with various other methods of activating this special material and find that it responds to most of them, so that we are convinced the material has special merit. We have passed various gases over the rotted coal both during the charring period and after the charring period, and find varying results, but apparently the best results are obtained by passing steam in large amounts over the highly heated char.

The material obtained in this way is a black, highly porous char which, when brought into contact with various liquids, such as oil or brown sugar solution, acts as a vigorous decolorizer and clarifier. It is much more active than fuller's earth or the various decolorizing chars we have been able to secure on the market, clarifying liquids to a greater extent and at the same time permitting of rapid filtration. Apparently there is some special merit in the particular material used, as the same results are by no means obtained from other well known materials when given the same treatment. For example, ordinary coal is practically inert as a decolorizing medium when it is subjected to the treatment described. Ordinary wood charcoal is an extremely poor decolorizing medium, whereas this rotted coal may be made into fairly good decolorizing material (about like fuller's earth) by simply passing it through a kiln.

We have produced the kilned product on a commercial scale by simply passing the rotted coal slowly through a hot zone in the kiln. And we have made the steam blown material by taking this kilned product and blowing highly superheated steam through it for several hours while it was maintained at about 1800 degrees Fahrenheit in a closed vessel. There is no apparent reason for doubting that this highly valuable product may be manufactured commercially by passing rotted coal through a kiln, allowing the red hot char to drop into a heat insulated chamber and there subjecting it to the action of highly superheated steam. Apparently there is enough fuel value in the volatile matter of the rotted coal to take care of all the heat requirements enumerated, especially when it is considered that considerable hot water gas will be generated by the contact of the hot char with the hot steam. The

heat derived from the volatile matter of the 5  
rotted coal is sufficient to take care of the  
heat requirements of the kiln. We find that  
it is generally not worth while to crush the  
rotted coal prior to kilning it, as it is of a  
friable nature and breaks up in the kiln so  
that there are few pieces left larger than  
an inch in through dimension when the char  
is discharged. A crusher can be used to re- 10  
duce the size of the finished material if  
desired.

We have tested this activated char against  
the various materials on the market and find  
it better than any of them; that is, it will  
15 decolorize more oil or sugar solution, the  
various materials all being sized to the same  
size and the other conditions—temperature,  
length of contact with the liquid, rate of  
mixing, etc.,—being equal. We have also  
20 regenerated this material after it had been  
used for decolorizing, and find it may be  
brought to approximately its original ac-  
tivity by simply passing it again through  
a red hot kiln.

25 It is obvious that where the small amount  
of ash in the activated char is objection-  
able, it may be leached out by subjecting  
the char to the action of chemical reagents,  
hydrochloric acid, for example. This will  
30 be necessary only in special cases, the ash  
having no harmful effect in many uses,  
such, for example, as the clarifying of oils.

While we have described this invention  
as applying to decolorizing of liquids, it  
35 will also be understood that the material  
may also be used for absorbing gases, and  
for any of the uses to which ordinary ac-  
tivated char is put.

What we claim is:

40 1. A filtering and decolorizing material  
consisting of charred rotted coal which has  
been subjected to the action of steam.

2. A filtering and decolorizing material  
consisting of activated charred rotted coal.

3. A filtering and decolorizing material 45  
consisting of charred rotted coal which has  
been subjected to the activating action of  
superheated steam.

4. The method of making decolorizing 50  
material, which consists in charring rotted  
coal by slowly passing it through a rotating  
kiln while subjecting it to a charring tem-  
perature, and then subjecting the hot rotted  
coal to the action of superheated steam.

5. The method of making decolorizing 55  
material, which consists in charring rotted  
coal, and subjecting the charred product,  
unmixed with other material, to the action  
of superheated steam.

6. The method of making decolorizing 60  
material, which consists in charring rotted  
coal unmixed with other material by slowly  
passing it through a rotating kiln while  
subjecting it to a temperature of about 1800  
degrees Fahrenheit, and conserving the heat 65  
of the charring process by blowing the rotted  
coal while hot with highly superheated  
steam.

7. The method of making decolorizing 70  
material, which consists in charring rotted  
coal, by passing it through a rotating kiln  
while subjecting it to a charring tempera-  
ture and then subjecting the hot rotted coal  
to the action of a flow of highly heated 75  
fluid.

In testimony whereof, we have hereunto  
subscribed our names this 31 day of May,  
1918.

HUGH RODMAN.  
EARL E. BOREN.

Witnesses:

R. L. KENT,  
ANNA CLOHERTY.